

Sept. 23, 1930.

G. H. CLARK

1,776,619

SILENT GEARS, ETC., AND METHOD OF MANUFACTURE

Filed Sept. 22, 1927



Fig. 2. Fig. 3.



Fig. 4.



Inventor:  
George H. Clark

By Dyerforth, Inc., Chittorgarh, W. Va.  
Attest:

## UNITED STATES PATENT OFFICE

GEORGE H. CLARK, OF CINCINNATI, OHIO, ASSIGNOR TO THE FORMICA INSULATION COMPANY, OF CINCINNATI, OHIO, A CORPORATION OF OHIO

## SILENT GEARS, ETC., AND METHOD OF MANUFACTURE

Application filed September 22, 1927. Serial No. 221,301.

This invention relates particularly to gear-wheels of the silent gear type having non-metallic teeth. Such gears are, at the present time, manufactured from various non-metallic substances. A highly satisfactory laminated product for the purpose is composed of cloth, or canvas, impregnated with a varnish of bakelite, redmanol, or other phenolic condensation product, the mass being compacted and hardened under heat and pressure.

One of the main difficulties with the use of a laminated product of the character mentioned for gear-blanks, or gears, is the tendency of the disk to become loose on the shaft. This is particularly true, when the gear is forced onto the shaft under heavy pressure, which may unintentionally exceed the elastic limit. In such a case, the material will cold-flow and the gear will loosen from the shaft.

Attempts have been made to overcome the difficulty mentioned by molding within the laminated disk a complete metal bushing, but this adds considerably to the cost of the gear-blank, and requires machining.

In accordance with the present invention, disks of bakelite-impregnated fabric are perforated and assembled in a special manner and have associated therewith stamped metal rings which are so related to the stack of fabric disks that a gear-blank may be formed in an economical manner in a heated hydraulic press, such gear-blank having embedded in its hub-portion the metallic disks so firmly anchored to the non-metallic body as to provide a reliable connection between the gear-blank and a shaft when a press-fit is effected.

The product and method of producing the same are illustrated in the accompanying drawing, in which—

Fig. 1 depicts several series of annular bakelized fabric disks adapted to form a gear-blank; Fig. 1<sup>a</sup>, a series of metallic washers adapted to be placed within the stack of fabric disks and molded therewith to form the gear-blank; Fig. 2, a perspective view of the fabric disk provided with a perforation of approximately the size of the shaft upon which the gear-blank is to be mounted;

Fig. 3, a perspective view of a fabric disk having a perforation of a size adapted to admit a metallic washer; Fig. 4, a perspective view of one of the metallic washers employed; Fig. 5, a sectional view of a finished gear; and Fig. 6, a broken base view of a finished gear-blank, shown partly provided with teeth.

Referring to Fig. 2, A designates a fabric disk impregnated with a solution of a phenolic condensation product, such as bakelite, the disk being provided with a central perforation A' which is somewhat smaller than the shaft on which the gear-blank is to be mounted.

Referring to Fig. 3, A<sup>2</sup> designates a similar disk, but having a perforation A<sup>3</sup> large enough in diameter to admit a metallic washer.

Referring to Fig. 4, B designates a metallic washer having a perforation B' of about the size of a shaft upon which the gear-blank is to be mounted and having an external diameter corresponding with the diameter of the perforation A<sup>3</sup>. The metallic disk B is cut or nicked at its circumferential portion, as indicated at B<sup>2</sup>.

In Fig. 1<sup>a</sup> is shown four of the metallic washers B, which is the number preferably used in connection with the fabric disks shown in Fig. 1.

In the diagrammatic view shown in Fig. 1, the disks A and A<sup>2</sup> are assembled in groups. For convenience, the groups are bracketed and the number of disks in each group is applied to the corresponding bracket.

The disks shown in Fig. 1 are arranged in the same relation in which they enter into the finished gear shown in Fig. 5, the finished gear being designated C. Thus, reading from right to left on Fig. 1, there are six of the blanks A; then six of the blanks A<sup>2</sup>; then one of the blanks A; then three of the blanks A<sup>2</sup>. The further arrangement will be understood from the diagram itself.

It will be noted that there are four groups, each containing three of the disks A<sup>2</sup>. Each of these four groups of three blanks receives or houses one of the metallic washers B in the

assembly of the pack for insertion into the mold of the hydraulic press.

After a suitable assembly of fabric disks and metallic washers has been introduced into the mold, the gear-blank is molded under heat and pressure, such as is ordinarily employed for producing laminated phenolic condensation products. A suitable pressure is about two thousand pounds per square inch, and a suitable temperature is about 175° C. The article preferably is maintained under heat and pressure until the phenolic condensation product has been converted to the final infusible and substantially insoluble condition. Ordinarily, the hot-pressing operation will require from ten to forty-five minutes, depending upon the size of the gear-blank, the temperature employed, etc.

The dies may be of suitable shape to produce the form of gear-blank indicated in Fig. 5. After the blank has been produced, the teeth may be cut, as in the case of an ordinary metal gear.

It will be noted that the use of the fabric disks arranged in the manner shown at the right-hand portion of Fig. 1 enables the dies to form the recess C' at one side of the gear-blank. Also, the dies, when this particular arrangement is employed, effect a certain amount of dishing of the washers B, and this tends to strengthen the bond between the metal washers and non-metallic body of the gear-blank.

It has been found in practice that metallic washers may in this manner be introduced into a gear-blank in such manner as to become virtually integral with the gear-blank; and when a gear-blank thus constructed is pressed onto a shaft under pressure of several tons, the gear-blank becomes so firmly fixed upon the shaft that there is no liability of its working loose. The gear-blank is shown provided with a central perforation C<sup>2</sup> to receive the shaft. This preparation may represent the bore of the gear-blank after it has been forced onto a shaft. That is, the finished gear-blank may have a bore represented by the diameters of the perforations A' and B'; or, if desired, the bore of the press-blank may be trimmed by means of a boring tool, although ordinarily this is unnecessary.

The foregoing detailed description has been given for clearness of understanding only, and no unnecessary limitations should be understood therefrom.

What I regard as new, and desire to secure by Letters Patent, is:

1. The process of producing a gear-blank which comprises: placing in a mold an assembly comprising annular disks of fabric impregnated with a phenolic condensation product, and metallic washers, some of the fabric disks having larger perforations than the others and serving to house said wash-

ers; and consolidating the assembly under heat and pressure.

2. The process of producing a gear-blank which comprises: assembling groups of fabric disks having bores of relatively small diameter and interspersed groups of fabric disks having bores of relatively large diameter and metallic washers housed within some of the larger bores; and consolidating the assembly under heat and pressure. 70

3. The process of forming a gear-blank which comprises: assembling alternating groups of disks impregnated with a binder, said groups having bores of different diameters and metallic washers housed in some of the larger bores, the outer groups at the ends of the assembly having small bores; and molding the assembly under heat and pressure. 75

4. The method of forming an article of the character described which comprises: assembling groups of fabric disks, impregnated with a phenolic condensation product, said groups having bores of different diameters and being arranged in alternation, and introducing metallic washers within the bores of intermediate groups of large diameter, the assembly providing an end group of disks having bores of small diameter and an adjacent group of disks having bores of large diameter; and subjecting the assembly to heat and pressure in a mold adapted to dish the body of the article at one side. 85

5. An article of the character set forth consisting of interspersed groups of fabric disks impregnated with a phenolic condensation product, said groups having bores of different diameters and metallic washers housed in some of the larger bores, all of said groups being consolidated under heat and pressure into an integral body within which said metallic washers are embedded, the inner circumferences of said metallic washers forming a part of the bore of the consolidated body. 100

GEORGE H. CLARK.

110

115

120

125

130